

July 30, 1935.

A. F. BRADLEY

2,009,573

## APPARATUS FOR DRY GALVANIZING WIRE

Filed June 21, 1933



Albert F. Bradley.

By Charles F. Wells

Atlys.

## UNITED STATES PATENT OFFICE

2,009,573

## APPARATUS FOR DRY GALVANIZING WIRE

Albert F. Bradley, Sterling, Ill., assignor to North-western Barb Wire Company, Sterling, Ill., a corporation of Illinois

Application June 21, 1933, Serial No. 676,768

5 Claims. (Cl. 91—12.2)

This invention relates to a method of and apparatus for dry galvanizing wire and other strip material of ferrous metal, such as iron or steel. The operation of dry galvanizing is frequently referred to as sherardizing, the principles of which are fairly well known. Sherardizing, however, has not heretofore been satisfactorily applied to wire, to the best of my knowledge.

According to the present invention, wire is drawn through a stationary bed of zinc dust, or other dust containing a large proportion of metallic zinc, at a temperature below that at which fusion and coalescence of the zinc particles results and above that at which cementation of the metallic zinc with the metal of the wire commences. The wire is drawn continuously through the heated bed of zinc dust and the zinc dust locally agitated so as to increase the contact of the dust with the wire and effect the desired degree of sherardizing during a single travel of the wire through the bed.

It is therefore an important object of this invention to provide a relatively inexpensive and efficient method of sherardizing strip material, such as wire, and to provide an apparatus particularly well adapted for the carrying out of such method.

Other and further important objects of this invention will be apparent from the disclosures in the specification and the accompanying drawing.

This invention (in a preferred form) is illustrated in the drawing and hereinafter more fully described.

On the drawing:

Figure 1 is a longitudinal, broken sectional view of apparatus embodying the principles of my invention and suitable for carrying out my method of sherardizing wire.

Figure 2 is a sectional view taken substantially on line II—II of Fig. 1 with parts omitted.

As shown on the drawing:

The reference numeral 10 indicates generally a furnace or retort supported upon legs or standards 11 which may be suitably braced by transverse angle irons 12 and 13 and inclined angle irons 14. The furnace or retort 10 is provided with a fire box 15 extending the full length thereof. Said furnace may be suitably fired as by means of oil or the like introduced through a nozzle 16 positioned at an opening 17 in one end of the furnace housing. Oil may be supplied to the nozzle 16 through a connecting pipe 18 and air or steam through a valved pipe 19.

An arched metallic plate 20 serves as the ceiling of the fire box 15 and to divide the fire box

from an upper chamber 21 that is substantially closed from the air by means of a top plate 22, side plates 23 and 24, a front plate 25 and a rear plate 26. Said front and rear plates 25 and 26, respectively, are provided with aligned apertures 27 and 28, respectively, through which strands of wire 29 or other strip material of ferrous metal may be passed for passage through a bed 30 of zinc dust contained within said chamber 21. Within said chamber 21 and supported from the plate 26 thereof are a plurality of baffles 32 and 33 which are slotted to provide guides for the strands 29 and which also serve to prevent the carrying along of the zinc dust with the strands of wire as they are pulled in the direction indicated by the arrow in Fig. 1. Dependent baffles 34 and 35 are likewise supported from the top plate 22 of said chamber 21 to serve the same purpose and also to provide bearings as at 36 and 37, respectively, for shafts 38.

Said shafts 38 extend substantially the full length of the chamber 21 and project through the rear end wall 26 thereof for connection by means of a plate 39 with a rocker arm 40. Said rocker arm 40 is mounted about a fulcrum point 41 provided by a bracket 42 that extends from a stand 43 mounted on said top plate 22. An eccentric 44 is suitably mounted on said stand 43 and is connected by means of a link 45 to one end of the rocker arm 40. Said eccentric 44 may be driven by any suitable means (not shown).

Each of the shafts 38 is provided with a plurality of rake-like members 46, fixedly secured at spaced intervals along said shafts and having downwardly extending tines 47 that dip below the surface of the bed 30. Said tines 47 may also suitably be provided with short transversely extending pins 48 to increase the agitating effect of the movement of the rake-like members 46 on the bed of zinc dust. The positions of the apertures 27 and 28 and of the dependent tines 47 of the rake-like members 46 are so arranged that the strands of wire 29 pass between adjacent tines 47 and in close proximity thereto. Consequently, the reciprocation of the rake-like members 46 effects a thorough agitation of the zinc dust in the bed 30 with resulting increased contact of the zinc dust with the moving wire strands. The rake-like members 46, together with the baffles 32, 33, 34 and 35 substantially prevent the carrying along of the zinc dust with the moving wires and also prevent the building up of the bed of zinc dust at any one spot.

Charging man holes 50 and 51 are provided in

the top plate 22 for introducing additional zinc dust into the chamber 21.

In operation, the combustion chamber 15 is heated to the desired temperature by the combustion of oil or other fuel introduced through the opening 17, together with sufficient air to support combustion. When the bed of zinc dust has reached the desired temperature, which should be below that at which the zinc particles will fuse and coalesce and above that at which cementation of the zinc with the metal of the wire will commence, the strands of wire 29 are drawn through the bed and the reciprocating apparatus started in motion to keep the bed thoroughly agitated and to increase the contact of the zinc dust particles with the wires. The temperature and time of travel of the wire through the bed of zinc dust are so controlled and regulated that the desired degree of sherardizing or dry galvanizing of the wire will be effected.

The wire may enter the zinc dust bath cold, but is preferably hot. For example, the wire may be passed in at annealing temperatures, around 1400 to 1600° F., and the sensible heat thereof utilized to effect the sherardizing step. The temperature at which proper sherardizing takes lies between about 650 and 750° F. To obtain these temperatures, either the wire or the zinc dust bath, or both, should be heated, the temperatures to be employed depending in part upon the speed of travel of the wire through the furnace.

It will be understood that instead of an oil or gas fired retort, superheated steam or other fluid heating means, or electrical heating means, may be employed. One of the important features of my invention is the close control of the temperature at which the bed of zinc dust is maintained in order to produce the desired character and degree of cementation of the zinc with the metal of the wire being passed through the apparatus. Another important feature of the invention is the provision of reciprocating agitating means in close proximity to the moving strands of wire, with the motion of the agitating means parallel to the strands of wire. By this means, the forming of voids in the bed of zinc dust or the building up of the bed locally to uncover any portion of the wire strands is avoided and very efficient contact between the zinc dust and the wire strands is insured.

While the bed of material has been referred to as consisting of zinc dust, it will be understood that commercial "blue dust", a byproduct in the usual method of smelting zinc, is a material that is generally used in the sherardizing process. In any event, the term "zinc dust" is intended to cover any of the various forms of zinc containing dust that are suitable for sherardizing operation. In general, such dusts contain approximately 85 to 90% of metallic zinc, with 5 to 8% of zinc oxide. As is well known, the use of a mixture of used and new dust, carefully freed from iron and oxide particles, is generally preferred in sherardizing processes.

Temperatures may, of course, be used such that the individual particles of zinc while in contact with the wire or strip material will be at an incipient melting stage, but actual fusing down and coalescing of the particles of zinc must be avoided if the best results are to be obtained. The temperature provided depends somewhat upon the composition of the zinc dust used, as well as upon the speed of travel of the wire through the

furnace, but in general the temperature of the zinc dust bath should be between about 650 and 800° F. As previously pointed out, the bath of zinc dust may be at a lower temperature, or even cold, if the wire is sufficiently hot when it enters the bath.

Air is substantially excluded from the chamber containing the zinc dust in order to prevent oxidation of the metal of the wire or the zinc. This is accomplished by making the apertures 27 and 28, through which the wire strands pass, comparatively small.

I am aware that many changes may be made and numerous details of construction may be varied through a wide range without departing from the principles of this invention, and I, therefore, do not purpose limiting the patent granted hereon otherwise than necessitated by the prior art.

I claim as my invention:

1. Apparatus for sherardizing wire, comprising a retort having a lower combustion chamber and an upper separate chamber for containing a bed of zinc dust, agitating means mounted in said upper chamber and having fingers extending into said bed of zinc dust, there being apertures in the end walls of said upper chamber for the passage of wires through said bed of zinc dust and means for reciprocating said fingers in directions parallel to said wires.

2. In an apparatus for "dry" galvanizing wire, a substantially closed receptacle for containing a bed of zinc dust, the end walls of said receptacle having apertures for the passage of wires therethrough, rakes having tines extending into said bed of zinc dust and in close proximity to said wires and means for reciprocating said rakes.

3. Apparatus for dry galvanizing a plurality of wires in one operation comprising a heating chamber, an elongated treating chamber thereabove in thermal contact therewith adapted to contain a bed of galvanizing dust, means for drawing wires through said chamber, rakes in said chamber and means for reciprocating said rakes longitudinally in the chamber for agitating the bed therein to insure contact of the wires with the bed.

4. Apparatus for sherardizing wire comprising a retort having a lower combustion chamber and an upper chamber sealed therefrom in thermal relation therewith, a plurality of shafts slidably mounted from the top of said upper chamber, a plurality of rakes extending downwardly from said shafts into close proximity with the bottom of said chamber, baffles mounted in the bottom of said chamber, means for directing a plurality of wires through said chamber adjacent to said rakes and means for reciprocating said rakes longitudinally of said wires.

5. Apparatus for sherardizing a plurality of wires in one operation comprising a combustion chamber having an arched top, a second chamber above said combustion chamber in thermal contact therewith, said arched top of said combustion chamber forming an arched bottom for said second chamber, charging doors in the top of said second chamber, means for guiding a plurality of wires through said second chamber, and means comprising a plurality of reciprocally movable rakes in said second chamber for agitating material inserted through the charging doors.

ALBERT F. BRADLEY.